# EUROPEAN PATENT SPECIFICATION

(11) **EP 3 180 477 B1**
(45) Date of publication and mention of the grant of the patent: **01.05.2019**
(21) Application number: 15832527.4
(22) Date of filing: 13.08.2015
(51) Int. Cl.: E01C 13/08, D05C 17/02, A63C 19/04, E01C 5/18

(54) **ARTIFICIAL TURF WITH NON-GRANULAR DAMPING MATERIAL AND METHOD FOR MANUFACTURING SAME**
KUNSTRASEN MIT NICHTKÖRNIGEM DÄMPFUNGSMATERIAL UND VERFAHREN ZUR HERSTELLUNG DESSEN
GAZON ARTIFICIEL COMPORTANT UN MATÉRIAU D'AMORTISSEMENT NON GRANULAIRE ET SON PROCÉDÉ DE FABRICATION

(30) Priority: 13.08.2014 FI 20145715
(43) Date of publication of application: 21.06.2017
(73) Proprietor: Salmenautio, Hannu, 62900 Alajärvi (FI); Salmenautio, Timo, 62900 Alajärvi (FI); Salmenautio, Anne, 62900 Alajärvi (FI)
(72) Inventor: Salmenautio, Hannu, 62900 Alajärvi (FI); Salmenautio, Timo, 62900 Alajärvi (FI); Salmenautio, Anne, 62900 Alajärvi (FI)
(74) Representative: Papula Oy
(86) International application number: PCT/FI2015/050523
(87) International publication number: WO 2016/024044

(56) References cited:
- EP-A1- 2 679 723
- WO-A1-2009/011569
- WO-A2-2008/051073
- GB-A- 2 253 638
- JP-A- 2008 019 670
- US-A- 3 293 723
- US-A- 5 830 080
- US-A1- 2007 160 800
- US-A1- 2007 224 361
- US-A1- 2008 125 237
- US-A1- 2008 292 819
- US-A1- 2010 129 571
- US-A1- 2012 058 294

## Description

### FIELD OF THE INVENTION

The invention relates to an artificial turf, according to the preamble of claim 1, suitable for use as a sports surface. The invention further relates to a method for manufacturing an artificial turf according to the preamble of claim 7.

### BACKGROUND OF THE INVENTION

Artificial turf systems generally consist of a backing, a large number of artificial grass fibers attached to the backing, and a thick infill layer distributed on the backing between the grass fibers. The artificial grass fibers, which can be tufted or knitted to the backing or co-woven therewith, protrude substantially perpendicularly to the backing. These artificial grass systems generally have a granular infill layer of rubber granules, sand, or both. Sand is used for stabilization of the turf and elastic material is used to endow the turf with elasticity.

Depending on the circumstances of use, an artificial turf sports field can be exposed to moisture and temperature variations, UV light and abrasion due to the use of the field. Problems associated with known artificial turfs include wear and fibrillation of the grass, as well as low elasticity of the turf. The use of granular infill in an artificial turf system has a number of drawbacks. Not only is the installation of such an artificial turf sports field more labour-intensive, but an artificial turf system comprising granular infill material requires regular maintenance also after it has been installed.

In the past years a number of non-granular infill systems have been introduced as alternatives to artificial turf systems comprising granular infill material.

US 6753049 B2 discloses an artificial turf having fibrous, inherently damping material arranged between artificial grass blades and connected to the backing or the blades. The fibrous material can be arranged in the form of blades connected to the backing, or it can also take the form of a knit through which the artificial grass blades protrude and which can be formed integrally with the backing.

US 6955841 B2 discloses an artificial grass lawn with a base layer comprising a material having damping properties. The damping material can be in the form of a damping mat which is fixed to the base layer by means of artificial grass fibers. The damping material can be made of rubber or a synthetic foam product can be used.

US 8557363 B2 discloses an artificial grass turf carpet having a base layer comprising a plurality of synthetic base layer fibers attached to the ground structure and positioned between upstanding synthetic grass fibers. The base layer fibers are positioned so tight against one another and against adjacent grass fibers to provide a tightly packed base layer above which the grass fibers extend.

US 3293723 A discloses a method of making a pile fabric, such as artificial fur, wherein the pile portion of the fabric is prepared from a crimped thermoplastic continuous filament yarn, having nonuniform latent shrinkage characteristics. The yarn may consist of entirely uncrimped and entirely crimped continuous filaments or intermittently crimped filaments.

US 5830080 A discloses a golf practice tee device and a turf-simulating surface that simulates the properties of natural turf, the turf-simulating surface comprising a surface composite and a composite base. The surface composite includes a pile section, a lateral-strength fabric, and a plastic foam element. The composite base, which simulates the supporting properties of the deeper layers of natural soil, comprises a foamed-plastic composite.

US 20080125237 A1 discloses a golf mat and a method of manufacture thereof. The golf mat includes a backing and artificial grass fibers attached to the backing. The artificial grass fibers are divided into groups of at least two different kinds of fibers sewn through a common path in the backing. One of the kinds of fibers in each group is shaped to appear like a blade of natural grass, and the other kind of fiber is crimped so that the relaxed shape of the fiber is nonlinear.

EP 2679723 A1 discloses a composition and a method for treating synthetic turf in order to improve ball roll characteristics of the turf and to improve the protection of the turf for wear and tear. The composition to be applied on the pile of the turf includes a flexible acrylic resin polymer, or a modified vinyl polymer or copolymer, together with a biocidal agent, surface active agent, and a de-foaming agent.

US 20070224361 A1 discloses a system and a method for spraying a liquid onto fibers in a synthetic turf. The method comprises the steps of providing a sprayer with a nozzle; positioning the nozzle at an angle with respect to the synthetic turf in a range of approximately 30°-60°; and spraying the liquid onto the monofilament fibers.

US 20100129571 A1 discloses an artificial turf and a method of making thereof, the artificial turf comprising a porous backing; yarn tufted into the backing, backloops of the yarn being arranged closely adjacent to a bottom face of the backing; and a porous coat of coating material deposited on the bottom face that bonds the tufted yarn to the backing. The viscosity of the deposited coating material causes it to resist flowing along the backing.

JP 2008019670 A discloses a method of reinforcing artificial turf, comprising a base fabric and lawn grass, wherein a water-resistant, curable liquid resin is applied onto the lawn grass, and the liquid resin is cured after having flowed down along the lawn grass and reached the base fabric.

WO 2008051073 A2 discloses an artificial grass fibre and an artificial lawn comprising the same. The artificial grass fibre comprises at least one material component, which imposes a permanent volume increase on the artificial grass fibre under the influence of an external stimulus, after an artificial mat has been provided with the artificial grass fibre. The artificial grass fibre is configured to foam and transform, for example, into a dampening layer after the manufacture of the lawn.

Drawbacks of the prior art are that the known damping materials are not sufficiently wear-resistant. As a consequence, the turf may have to be fixed or replaced after a relatively short time. Also, the elasticity of known damping base layers is reduced quite rapidly.

The normally used pile yarns are relatively thin and therefore the base fibers have to be tightly packed in order to allow the layer to withstand the weight of the players and to sufficiently stabilize the turf. This is because the current production methods for artificial turfs are not readily suitable for tufting or weaving yarns above certain thickness. Tightly packed base layer fibers do not allow the studs of a football shoe to penetrate into the base layer. Instead, the grip of the football shoes on the turf is poor thus causing a danger of injury to the players.

The inventors have therefore recognized the need for a new type of artificial turf comprising non-granular damping material having improved elasticity, stability and wear-resistance.

### PURPOSE OF THE INVENTION

The purpose of the invention is to provide a new type of artificial turf that can be used without granular infill or can be used with reduced granular infill. Specifically, the purpose of the invention is to provide an artificial turf with improved properties, e.g. improved elasticity and wear-resistance.

### SUMMARY

The present invention relates to an artificial turf having the features of claim 1.

The present invention further relates to a method for manufacturing an artificial turf having the features of claim 7.

Further preferred embodiments are defined by the features of dependent claims 2-6,8-13.

The base and grass fibers of the artificial turf are reinforced by non-granular infill material applied as a coating on individual fibers. In one embodiment the base and grass fibers have mutual points of contact and the coating binds the reinforced parts of the base and grass fibers together at the points of contact. As a result, a resilient layer is formed at the foot of the grass fibers, comprising the reinforced parts of the base and grass fibers including the coating of infill material applied on the surface of the fibers. In one embodiment non-reinforced parts of the base fibers extend above the resilient layer.

The resilient layer is porous and contains spaces between the fibers. In addition, the reinforced fibers are bound together at their points of contact. This kind of structure gives the layer good elasticity and improves the layer's ability to return to its original shape after applied physical stress.

The resilient layer is water-permeable and allows water to penetrate through the layer. In known artificial turfs, the attachment of the fibers is normally improved by applying adhesive as a non-permeable layer on the second side of the backing. This adhesive layer contains holes at certain intervals to allow water to penetrate the adhesive layer. Said holes are easily clogged up, thereby reducing water-permeability over time. The resilient layer according to the present invention improves attachment of the fibers into the backing. It is therefore not necessary to apply a separate non-permeable adhesive layer on the second side of the backing. Thus, the artificial turf according to the present invention is water-permeable throughout the turf, which reduces risk of clogging. Also, the water is able to quickly penetrate the turf.

The structure of the resilient layer allows the layer to maintain its elasticity for a long period of time. The durability of the reinforced base fibers is better than the durability of corresponding non-reinforced base fibers, making the turf wear-resistant. The damping effect caused by the layer of reinforced fibers is uniform over the entire turf. Also, the behavior of the ball on the surface is similar to the behavior of the ball on natural grass.

The thickness of the coating applied on the surface of the fibers depends on the application and the infill material used. In one embodiment the coating is not uniform over the surface of the fibers. In the final product, part of the length of the grass fibers and at least part of the length of the base fibers is covered by the coating. In one embodiment part of the length of the grass fibers and at least most of the length of the base fibers is covered by the coating. In one embodiment, the whole length of the base fibers is covered by the coating.

In one embodiment, the shock absorption of the artificial turf is from 30% to 70%, as measured according to standard EN 14808 (Surfaces for sports areas. Determination of shock absorption) using the Artificial Athlete 2A equipment. Shock absorption is a measure of resiliency of the layer. In one embodiment, the deformation of the artificial turf according to the present invention is from 4 to 12 millimeters, as measured according to standard EN 14809 (Surfaces for sports areas. Determination of vertical deformation) using the Artificial Athlete 2A equipment. Deformation is a measure of surface stability. The shock absorption and the deformation are measured for the turf comprising no granular infill material and placed on concrete base. In other words, good shock absorption and deformation values are achieved without the use of granular infill. In addition, the turf according to the present invention maintains good shock absorption and good deformation values for many years.

The layer of reinforced fibers is able to maintain the grass fibers in an approximately vertical orientation in use without requiring the provision of a granular infill. Hence, the layer of reinforced base fibers is capable of totally replacing granular infill which is traditionally used in artificial turf systems. However, depending on the application, the turf may also be supplied with granular infill. Granular infill may assist e.g. in stabilizing turfs that have to withstand the weight of heavy vehicles. In one embodiment the artificial turf according to the present invention comprises an infill layer of rubber granules, sand, or both.

In one embodiment of the present invention the artificial turf is installed on a firm surface. In one embodiment the artificial turf is installed on a separate resilient base layer. The resilient base layer can be of any elastic material.

In one embodiment the base fibers are reinforced by heating them to a temperature near to or equal to the melting point of the raw material of the fibers, followed by rapid cooling. The heating causes the surface of the fibers to melt thereby reinforcing the structure of the fibers. The temperature and duration of the heat treatment is determined by the material of the fibers. In one embodiment the grass fibers are attached to the backing before the heat treatment so that the grass fibers are exposed to the heat treatment simultaneously with the base fibers. In one embodiment the grass fibers are attached to the backing after the heat treatment of the base fibers so that the grass fibers are not exposed to the heat treatment.

The backing can consist of one or more layers of woven or non-woven fabric each having a relatively open net structure. The open net structure of the backing comprises holes. In one embodiment the mesh of the fabric used as a backing is from 1 to 15 millimeters. The open net structure can be inherent to the fabric wherein pile yarns forming the grass and base fibers are attached by tufting. The open net structure of the fabric may also be formed by weaving while simultaneously co-weaving the pile yarns into the fabric. The backing comprises a first side and a second side. The pile yarns forming artificial grass and base fibers are attached to the backing so that they protrude from the backing to the direction of the first side. The second side is the side opposite to the first side.

In one embodiment, synthetic pile yarns forming the artificial grass and base fibers are attached to the backing by weaving or tufting. In one embodiment pile yarn is attached to the backing by traditional weaving or tufting techniques. Traditional weaving or tufting results in a turf wherein the distance between successive pile yarns in a row is constant. In one embodiment, pile yarns are attached to the backing by Matrix weaving technique or Matrix tufting technique. In Matrix technique, the distance between successive pile yarns in a row is not constant. For instance, four short stitches are followed by one longer stitch in a row. The number of successive short and long stitches may vary. In one embodiment, three short stiches are followed by one longer stitch in a row. As a consequence, the pile yarns are not uniformly distributed over the surface of the turf but the turf comprises discrete dense groups of pile yarns called bundles. The distance between pile yarn bundles is longer that the distance between successive pile yarns in a row. As a result, the turf is resilient and behavior of the ball on the surface is closer to natural grass.

In one embodiment the pile yarns are fixed to the backing by means of an adhesive, such as polyurethane or latex. In one embodiment the pile yarns are not fixed to the backing by means of an adhesive. In one embodiment the pile yarns are fixed to the backing by a water-permeable layer of adhesive.

In one embodiment, the pile yarns are attached by tufting. In one embodiment, the gauge of the tufting machine is 4.67 mm (3/16") and the number of stiches in a row is from 15 to 30 per 10 centimeters. In one embodiment, the gauge of the tufting machine is 3.97 mm (5/32") and the number of stiches in a row is from 15 to 30 per 10 centimeters. In one embodiment, the gauge of the tufting machine is 7.9 mm (5/16") and the number of stiches in a row is from 10 to 30 per 10 centimeters. In one embodiment, the gauge of the tufting machine is 15.8 mm (5/8") and the number of stiches in a row is from 10 to 30 per 10 centimeters. In one embodiment, the gauge of the tufting machine is 9.53 mm (3/8") and the number of stiches in a row is from 10 to 30 per 10 centimeters. In one embodiment, the gauge of the tufting machine is 19.6 mm (3/4") and the number of stiches in a row is from 10 to 30 per 10 centimeters. The gauge of the tufting machine refers to the number of needles per millimeter (inch) and corresponds to the number of stitches per millimeter (inch) in a direction perpendicular to rows. The number of stitches in a row is affected by the size of the needles in the tufting machine and the thickness of the yarn. In one embodiment, the pile yarns are attached by weaving and the distance between successive pile yarns in a row is from 1 to 10 millimeters and the distance between adjacent rows is from 1 to 10 millimeters. In one embodiment, the pile yarns are attached by Matrix weaving and the gap between successive pile yarn bundles in the direction of rows is from 5 to 20 millimeters and the gap between adjacent pile yarn bundles in the direction perpendicular to rows is from 5 to 20 millimeters. In one embodiment, the pile yarns are attached by tufting and the distance between successive pile yarns in a row is from 3 to 15 millimeters and the distance between adjacent rows is from 3 to 25 millimeters. In one embodiment, the pile yarns are attached by Matrix tufting and the gap between successive pile yarn bundles in the direction of rows is from 5 to 15 millimeters and the interval between adjacent pile yarn bundles in the direction perpendicular to rows is from 5 to 20 millimeters.

Both the grass and base fibers can comprise straight or crimped yarns or a combination of straight and crimped yarns. The yarn may also be made of a raw material that is crimped under certain reaction conditions, e.g. when the yarn is exposed to heat. The raw material of pile yarn can be, for instance, polyethylene, polypropylene, nylon, or any other suitable plastic material. Both the grass and base fibers may comprise fibers made of different materials. In one embodiment the height of grass fibers is from 30 to 75 millimeters and preferably from 30 to 40 millimeters. In one embodiment the height of straight base fibers is from 20 to 75 millimeters and preferably from 20 to 30 millimeters. In one embodiment the height of crimped base yarns is from 20 to 75 millimeters and preferably from 20 to 30 millimeters. In one embodiment, the height of the base fibers is lower than the height of the grass fibers. In one embodiment, the height of the base fibers is equal to the height of the grass fibers.

In one embodiment of the present invention the artificial grass fibers comprise monofilament pile yarn. In one embodiment of the present invention the artificial base fibers comprise monofilament pile yarn. In one embodiment of the present invention the artificial grass fibers comprise multifilament pile yarn. In one embodiment of the present invention the artificial base fibers comprise multifilament pile yarn. In one embodiment pile yarn is produced from single filaments by winding from 1 to 40, preferably from 1 to 20, and most preferably from 6 to 10 filaments together. In one embodiment the dtex of the individual filament ranges between 500 and 4000 dtex, and preferably between 800 and 3000 dtex. Dtex is a measure of linear mass density of fibers and is defined as the mass in grams per 10000 meters.

In one embodiment the artificial grass fibers comprise fibrillated pile yarn. In one embodiment the artificial base fibers comprise fibrillated pile yarn. Fibrillated pile yarn is produced in the form of a band having a width of 10-15 mm, followed by incision thereof (fibrillation). In one embodiment the dtex of fibrillated pile yarn ranges between 1500 and 17000 dtex, and preferably between 6000 and 12000 dtex. The artificial grass fibers or artificial base fibers may also comprise both monofilament or multifilament pile yarn and fibrillated pile yarn.

In one embodiment the turf is further processed after the formation of the resilient layer of reinforced base fibers by using different downstream processes. For example, the turf may be immersed in water or a suitable chemical. Alternatively, water or a suitable chemical may be sprayed on the turf. The turf may also be exposed to heat treatment. The purpose of the further processing steps may be to detach loose infill material from certain parts of the turf or to improve the adhesion of the infill material to the base fibers.

The non-granular infill material is extruded from the second side of the backing, i.e. from the side opposite the grass and base fibers. The extrusion from the rear side of the backing allows applying the infill material only to the base fibers and the lower parts of the grass fibers, thereby leaving the upper parts of the grass fibers, and optionally the upper parts of the base fibers, untreated.

In one embodiment, the non-granular infill material is applied on the rear side of the backing and pressed through the holes in the backing so as to form a porous layer of non-granular infill material at the foot of the grass fibers. In one embodiment the non-granular infill material is pressed by a press roll through the holes in the backing into the spaces between grass fibers. The mixing of the infill material with the base fibers and porosity of the resulting resilient layer can be improved by application of pressurized air after the application or extrusion of the non-granular infill material.

In one embodiment of the present invention, the non-granular infill material comprises elastomer. In this specification, the expression "elastomer" should be understood as a polymer having both viscosity and elasticity. In one embodiment the elastomer is thermoset elastomer. In one embodiment the elastomer is thermoplastic elastomer. In one embodiment the elastomer is fluent. In one embodiment the fluent elastomer is in liquid form. In one embodiment the fluent elastomer is in a form of a gel. In one embodiment of the present invention fluent elastomer is extruded from the second side of the backing through the holes in the backing into the spaces between the grass fibers and base fibers, and the elastomer is cured or vulcanized to form a resilient and water-permeable layer of reinforced fibers. The curing or vulcanization can be achieved e.g. by heat, chemical additives or electron beams or by exposure to air or water. In one embodiment, curing or vulcanization is performed at room temperature.

In one embodiment of the present invention, the non-granular infill material consists of elastomer.

In one embodiment the elastomer is silicone, styrene-butadiene rubber (latex), polyacrylic rubber or polyurethane. In one embodiment the elastomer is silyl modified polymer. In this specification, the expression silicone should be understood as a polymer that includes silicon, carbon, hydrogen, oxygen and optionally other elements. In one embodiment, silicone is silicone oil, silicone grease, silicone rubber, silicone resin or silicone caulk. In one embodiment the silicone is polysiloxane or polydimethylsiloxane. In one embodiment the silicone is polyxane. In one embodiment the elastomer is an adhesive. The choice of the elastomer is determined by the raw material and the properties of the fibers.

In one embodiment of the present invention the fluent elastomer is allowed to penetrate in between the base fibers from the rear side of the backing by immersing the artificial turf in a container containing liquid elastomer of low viscosity. The elastomer is thus absorbed into artificial turf from the rear side. The height of the forming resilient layer depends on the viscosity of the elastomer and the time of the procedure.

In one embodiment additives may be added to the elastomer before applying the elastomer on the surface of the fibers. The additives may be used to improve the properties of the artificial turf e.g. by improving resistance to UV light, by reducing friction or by adding scent of natural grass.

In one embodiment the height of the resilient and water-permeable layer is from 2 to 50 millimeters, preferably from 5 to 30 millimeters, and most preferably from 10 to 30 millimeters.

In one embodiment the grass fibers extend from 5 to 25 millimeters above the resilient and water-permeable layer. In one embodiment the top parts of the base fibers extend above the resilient layer. The height of grass fibers, base fibers and resilient layer is determined by the application of the turf, i.e. whether the turf is used as a sports field, in landscape use or for children's play-ground.

In one embodiment the fibers consist of filaments and the number of filaments per square meter is from 90000 to 350000. In order to achieve adequate resiliency of the turf, the number of reinforced fibers per square meter does not need to be as high as the number of corresponding fibers that are not reinforced. In other words, the number of filaments per square meter does not need to be as high in the turf according to the present invention as the number of filaments that are not reinforced. The number of filaments in a turf without granular infill is typically from 300000 to 600000 per square meter. Because the number of filaments per square meter is lower in the present invention than with non-reinforced fibers, the resulting layer permits the studs of football shoes to penetrate into said layer thereby improving the grip of the football shoes on the turf. The layer of reinforced base fibers thus resembles natural soil.

The embodiments of the invention described hereinbefore may be used in any combination with each other. Several of the embodiments may be combined together to form a further embodiment of the invention. An artificial turf or a method for manufacturing an artificial turf, to which the invention is related, may comprise at least one of the embodiments of the invention described hereinbefore.

The turf according to the present invention allows omitting the use of granular infill which is easily displaced during use and maintenance and causes nonuniform damping over the turf. An advantage of the present invention is that the dampening effect is uniform over the whole surface of the turf. The turf is extremely wear-resistant because the resilient layer comprises reinforced base fibers. The resilient layer improves attachment of the fibers to the backing. Further, the elasticity of the elastomeric layer is maintained remarkably long. The porous structure of the turf allows good water-permeability which is maintained for years. The artificial turf according to the present invention therefore requires little maintenance, resulting in reduced costs. The performance of the turf is not dependent on regular maintenance, but stays constant over the years. In addition, recycling of the material of the artificial turf according to the present invention is easy.

An advantage is that the individual base fibers are reinforced by a coating of non-granular infill material surrounding the fibers. As a consequence, the base fibers need not be as tightly packed as without the reinforcing coating in order to achieve the same resiliency. The structure of the base layer thus allows the studs of football shoes to penetrate into the resilient layer in a similar manner as they would penetrate into natural soil. This brings about a good grip on the artificial turf. Also, the behaviour of the ball on the surface resembles the behavior of the ball on natural grass. This kind of structure is also able to efficiently dampen shocks during the game. An advantage is that the artificial turf is not heated in the sunshine to the same extent that an artificial turf containing granular infill.

### BRIEF DESCRIPTION OF THE DRAWINGS

The accompanying drawings, which are included to provide a further understanding of the invention and constitute a part of this specification, illustrate embodiments of the invention and together with the description help to explain the principles of the invention. In the drawings:
Fig. 1 is a cross-sectional view of an artificial turf according to one embodiment of the present invention,
Fig. 2 is a cross-sectional view of an artificial turf according to a second embodiment of the present invention,
Fig. 3 is a cross-sectional view of a reinforced grass fiber of the turf according to Figures 1 and 2 (III-III),
Fig. 4 is a cross-sectional view of a reinforced base fiber of the turf according to Figures 1 and 2 (IV-IV),
Fig. 5 is a top view of an artificial turf according to a third embodiment of the present invention, and
Fig. 6 is a top view of an artificial turf according to a fourth embodiment of the present invention.

### DETAILED DESCRIPTION OF THE INVENTION

Reference will now be made in detail to the embodiments of the present invention, examples of which are illustrated in the accompanying drawings.

The description below discloses some embodiments of the invention in such a detail that a person skilled in the art is able to utilize the invention based on the disclosure. Not all steps of the embodiments are discussed in detail, as many of the steps will be obvious for the person skilled in the art based on this specification.

For reasons of simplicity, item numbers will be maintained in the following exemplary embodiments in the case of repeating components.

Figures 1 and 2 are cross-sectional views of artificial turfs according to one and second embodiment of the present invention. The turf comprises a backing 1 having an open net structure. The backing 1 comprises a first side 11 and a second side 12. Pile yarn 14 simulating grass fibers 2 and base fibers 3 are attached to the backing 1 by tufting of weaving. In Figure 1, both the grass 2 and base fibers 3 are made of straight pile yarn 14 producing straight fibers. In figure 2, the grass fibers 2 are made of straight pile yarn 14 and the base fibers 3 are made of crimped pile yarn 14. The height 4 of the base fibers 3 is about half of the height 17 of the grass fibers 2. The height 4,17 of the base 3 and grass fibers 2 may vary depending on the embodiment and also the mutual relationship of their height can vary. For reasons of clarity, the distance between individual fibers 2,3 in the figure is relatively long. In practice, the fibers 2,3 can be attached to the backing 1 more densely. The fibers 2,3 extend upwardly from the backing 1 on the first side 11 of the backing 1. The grass 2 and base fibers 3 touch each other at mutual points of contact 9.

In Figures 1 and 2 parts 7 of the grass 2 and base fibers 3 have been reinforced by application of a coating 6 comprising non-granular infill material 5 on the surface of the fibers 2,3. The coating 6 has been applied by extruding non-granular infill material 5 from the second side 12 of the backing 1 so that the infill material forms a layer 8 of certain height 10. The height 10 of the layer 8 has been marked in the figure by a straight line. However, in practice the height 10 of the layer 8 is not constant throughout the layer 8 but varies from one position to another. For reasons of simplicity, the coating 6 has not been marked in the figure. The fibers 2,3 are reinforced by the coating 6 within the layer 8. The coating 6 makes the fibers 2,3 stronger and improves their elasticity. The coating 6 also binds the fibers 2,3 together at the points of contact 9 where the individual fibers 2,3 touch each other. The reinforced parts 7 of the grass 2 and base fibers 3 thereby form a resilient and water-permeable layer 8. The layer 8 comprises spaces 16 to allow water to penetrate the layer.

Figure 3 is a cross-sectional view of a reinforced grass fiber 2 of the turf according to Figures 1 and 2 (III-III). In other words, Figure 3 shows the horizontal cross-section of the grass fiber 2 within the resilient and water-permeable layer 8. The non-particular infill material 5 forms a coating 6 on the surface of the grass fiber 2. The thickness of the coating 6 material is not uniform over the surface of each individual fiber 2 but is varying. The thickness of the coating 6 depends on the orientation of the neighboring fibers 2,3. The coatings 6 of the neighboring fibers 2,3 may be combined together. The thickness of the coating 6 also depends on the thickness of the infill material 5 applied on the surface of the fibers 2. In Figure 3, the cross-section of the grass fiber 2 has a conically tapering and distorted shape. The grass fiber 2 can, however, have a cross-section of any other shape, e.g. rectangular, V shaped or rhombus shaped.

Figure 4 is a cross-sectional view of a reinforced base fiber 3 of the turf according to Figures 1 and 2 (IV-IV). In other words, Figure 4 shows the horizontal cross-section of the base fiber 3 within the resilient and water-permeable layer 8. The non-particular infill material 5 forms a coating 6 on the surface of the base fiber 3. The thickness of the coating 6 material is not uniform over the surface of each individual fiber 3 but is varying. The thickness of the coating 6 depends on the orientation of the neighboring fibers 3,2. The coatings 6 of the neighboring fibers 3,2 may be combined together. The thickness of the coating 6 also depends on the thickness of the infill material 5 applied on the surface of the fibers 3. In Figure 4, the cross-section of the base fiber 3 has a conically tapering and distorted shape. The base fiber 3 can however have a cross-section of any other shape, e.g. rectangular, V shaped or rhombus shaped.

Figure 5 is a top view of an artificial turf according to a third embodiment of the present invention. The turf has been manufactured by Matrix weaving technique. The backing 1 comprises an open net structure comprising holes 13. Only part of the net structure is shown in the figure. The pile yarn forming grass fibers 2 are attached to the backing 1 in rows 18 and at spaced intervals 15. For reasons of simplicity, base fibers 3 are not shown in the figure. The distance between successive grass fibers 2 in a row 18 is not constant. Four short stitches are followed by a longer one, thereby forming a larger gap 19 between successive grass fibers 2 in a row. The mutual distance between four adjacent rows 18 is constant, followed by a longer gap 19 between two adjacent rows 18. The grass fibers 2 located at an equal distance from adjacent grass fibers 2 form bundles 20 of grass fibers 2. One bundle 20 contains sixteen pile yarns forming grass fibers 2. These grass fiber 2 bundles 20 are separated from each other by a gap 19 of a longer distance than the distance of adjacent grass fibers 2 within a bundle 20.

Figure 6 is a top view of an artificial turf according to a fourth embodiment of the present invention. The turf has been manufactured by Matrix tufting technique. The backing 1 comprises an open net structure comprising holes 13. Only part of the net structure is shown in the figure. The pile yarn forming grass fibers 2 are attached to the backing 1 in rows 18 and at spaced intervals 15. For reasons of simplicity, base fibers 3 are not shown in the figure. The distance between successive grass fibers 2 in a row 18 is not constant. Four short stitches are followed by a longer one, thereby forming a larger gap 19 between successive grass fibers 2 in a row. The mutual distance between rows 18 of grass fibers 2 is constant. The grass fibers 2 in a row located at an equal distance from successive grass fibers 2 form bundles 20 of grass fibers 2. One bundle 20 contains four successive pile yarns in a row forming grass fibers 2. These grass fiber 2 bundles 20 are separated from each other by a gap 19 of a longer distance than the distance of adjacent grass fibers 2 within a bundle 20.

### EXAMPLES

### EXAMPLE 1 - Manufacturing artificial turf according to the present invention by Matrix tufting

An artificial turf was manufactured on a polypro-pene backing having an open net structure. The mesh of the backing was 3 millimeters. The dtex value of the pile yarn used in the current example was 2000. Straight pile yarn made of polyethylene was attached by tufting at spaced intervals to one side of the backing to provide artificial grass fibers. Four successive pile yarns in a row forming grass fibers were attached at intervals of 5 millimeters, followed by a longer gap of 10 millimeters. In addition, crimped pile yarn made of polyamide was attached by tufting at spaced intervals to the same side of the backing to provide artificial base fibers. Four successive pile yarns in a row forming base fibers were attached at intervals of 5 millimeters, followed by a longer gap of 10 millimeters. The height of the grass fibers, as measured from the backing, was 40 millimeters and the height of the base fibers was 30 millimeters. The fibers were attached so that they extend upwardly from the backing when the turf is in use. After tufting the yarns were fixed to the backing by adding a permeable layer of polyurethane adhesive on the second side of the backing. The amount of polyurethane per square meter was from 250 to 500 grams.

5000 grams per square meter silicone (polyoxane) was then applied on the rear side of the backing, i.e. the side opposite to the grass and base fibers. Silicone was extruded from the rear side of the backing through the holes in the backing into the spaces between the grass fibers and base fibers in order to mix the silicone with the fibers. The silicone thus formed a reinforcing coating on individual fibers. The length of the base and grass fibers was partly covered with the coating. The silicone coating extended from 25 to 30 millimeters upwards from the fabric. The reinforced base fibers thereby formed a resilient layer comprising holes and allowing water to penetrate through. The shock absorption of the turf was 50%, as measured according to standard EN 14808 using the Artificial Athlete 2A equipment. The deformation of the turf was 5.8 millimeters, as measured according to standard EN 14809 using the Artificial Athlete 2A equipment. The grass fibers of the turf manufactured according to this example extend over the resilient layer, and the layer is able to keep the grass fibers in an approximately vertical orientation in use without the provision of sand or rubber granules.

### EXAMPLE 2 - Manufacturing artificial turf according to the present invention by Matrix weaving

An artificial turf was manufactured by Matrix weaving, and the pile yarn forming the grass and base fibers were simultaneously attached. The resulting turf had a backing having an open net structure and the mesh of the backing was 1 millimeter. The dtex value of pile yarn used in the current example was 2500. Straight pile yarn made of polypropylene was attached by weaving at intervals of 9 millimeters to one side of the backing to provide artificial grass fibers. In addition, straight pile yarn made of polypropylene was attached by weaving at intervals of 9 millimeters to the same side of the backing to provide artificial base fibers. The height of the grass fibers, as measured from the backing, was 30 millimeters and the height of the base fibers was 20 millimeters. The fibers were attached so that they extend upwardly from the backing when the turf is in use. After weaving the yarns were fixed to the backing by adding a permeable layer of adhesive, i.e. 600 grams per square meter polypropylene dispersion.

800 grams per square meter polyurethane was then applied on the rear side of the backing, i.e. the side opposite to the grass and base fibers. Polyurethane was then extruded from the rear side of the backing through the holes in the backing into the spaces between the grass fibers and base fibers in order to mix the polyurethane with the fibers. The polyurethane thus formed a reinforcing coating on individual fibers. The length of the base and grass fibers was partly covered with the coating. The polyurethane coating extended approximately 20 millimeters upwards from the backing. The reinforced base fibers thereby formed a resilient layer comprising holes and allowing water to penetrate through. The shock absorption of the turf was 43%, as measured according to standard EN 14808 using the Artificial Athlete 2A equipment. The deformation of the turf was 4.2 millimeters, as measured according to standard EN 14809 using the Artificial Athlete 2A equipment. The grass fibers of the turf manufactured according to this example extend over the resilient layer, and the layer is able to keep the grass fibers in an approximately vertical orientation in use without the provision of sand or rubber granules.

It is obvious to a person skilled in the art that with the advancement of technology, the basic idea of the invention may be implemented in various ways. The invention and its embodiments are thus not limited to the examples described above; instead they may vary within the scope of the claims.

## Claims

1. An artificial turf comprising a backing (1) of open net structure, a plurality of artificial grass fibers (2) and a plurality of artificial base fibers (3), wherein said grass (2) and base fibers (3) are attached to the backing (1) and extend upwardly from the backing (1) when in use, and wherein the backing (1) comprises a first side (11) and a second side (12) opposite to the first side (11) and opposite the grass (2) and base fibers (3) **characterized in that** the base (3) and grass fibers (2) are reinforced by non-granular infill material (5), which comprises elastomer, as a coating (6) on each fiber (2,3) and covering part of the length of the grass fibers (2) and at least part of the length of the base fibers (3), and wherein the backing (1) comprises holes (13) for extruding the non-granular infill material (5) from the second side (12) of the backing (1) and wherein the reinforced parts (7) of the base (3) and grass fibers (2) form a resilient and water-permeable layer (8) which is attached to the backing (1) and over which the grass fibers (2) extend.

2. The artificial turf according to claim 1, wherein the base (3) and grass fibers (2) have mutual points of contact (9) and wherein the coating (6) binds the reinforced parts (7) of the base (3) and grass fibers (2) together at the points of contact (9).

3. The artificial turf according to claim 1 or 2, wherein the elastomer is silicone, styrene-butadiene rubber, polyacrylic rubber or polyurethane.

4. The artificial turf according to claims 1 to 3, wherein the height (10) of the resilient and water-permeable layer (8) is from 2 to 50 millimeters, preferably from 5 to 30 millimeters, and most preferably from 10 to 30 millimeters.

5. The artificial turf according to claims 1 to 4, wherein the grass fibers (2) extend from 5 to 25 millimeters above the resilient and water-permeable layer (8).

6. The artificial turf according to claims 1 to 5, wherein the fibers consist of filaments and the number of filaments per square meter is from 90000 to 350000.

7. A method for manufacturing an artificial turf, comprising the steps of:
- providing a backing (1) of open net structure comprising a first side (11), a second side (12) opposite to the first side (11), and a plurality of holes (13),
- attaching pile yarn (14) at spaced intervals (15) to the first side (11) of the backing (1) to provide artificial grass fibers (2) extending upwardly from the backing (1) when in use,
- attaching pile yarn (14) at spaced intervals (15) to the first side (11) of the backing (1) to provide artificial base fibers (3) extending upwardly from the backing (1) when in use, **characterized in that** non-granular infill material (5) comprising elastomer is extruded from the second side (12) of the backing (1) through the holes (13) in the backing (1) into the spaces (16) between the grass fibers (2) and base fibers (3) so that the non-granular infill material (5) is applied as a coating (6) on each fiber (2,3) in such a way that it covers part of the length of the grass fibers (2) and at least part of the length of the base fibers (3) and thereby reinforces said fibers (2,3), wherein the reinforced parts (7) of the base (3) and grass fibers (2) form a resilient and water-permeable layer (8) which is attached to the backing (1) and over which the grass fibers (2) extend.

8. The method for manufacturing an artificial turf according to claim 7, wherein the base (3) and grass fibers (2) have mutual points of contact (9) and wherein the coating (6) binds the reinforced parts (7) of the base (3) and grass fibers (2) together at the points of contact (9) .

9. The method according to claim 7 or 8, wherein fluent elastomer is extruded from the second side (12) of the backing (1) through the holes (13) in the backing (1) into the spaces (16) between the grass fibers (2) and base fibers (3), and the elastomer is cured or vulcanized to form the resilient and water-permeable layer (8) of reinforced fibers (2,3).

10. The method according to claim 9, wherein the elastomer is silicone, styrene-butadiene rubber, polyacrylic rubber or polyurethane.

11. The method according to claims 7 to 10, wherein the height (10) of the resilient and water-permeable layer (8) is from 2 to 50 millimeters, preferably from 5 to 30 millimeters, and most preferably from 10 to 30 millimeters.

12. The method according to claims 7 to 11, wherein the grass fibers (2) extend from 5 to 25 millimeters above the resilient and water-permeable layer (8).

13. The method according to claims 7 to 12, wherein the fibers consist of filaments and the number of filaments per square meter is from 90000 to 350000.

## Patentansprüche

1. Kunstrasen, umfassend eine Trägerschicht (1) mit einer offenen Netzstruktur, eine Vielzahl von Kunstgrasfasern (2) und eine Vielzahl von Kunstbasisfasern (3), wobei die Grasfasern (2) und Basisfasern (3) an der Trägerschicht (1) befestigt sind und sich im Gebrauch von der Trägerschicht (1) nach oben erstrecken, und wobei die Trägerschicht (1) eine erste Seite (11) und eine zweite Seite (12) gegenüberliegend zur ersten Seite (11) und gegenüberliegend zu den Grasfasern (2) und Basisfasern (3) aufweist, **dadurch gekennzeichnet, dass** die Basisfasern (3) und Grasfasern (2) durch nicht granuliertes Einfüllmaterial (5) verstärkt sind, das als eine Beschichtung (6) auf jeder Faser (2, 3) Elastomer umfasst und einen Teil der Länge der Grasfasern (2) und zumindest einen Teil der Länge der Basisfasern (3) bedeckt, und wobei die Trägerschicht (1) Löcher (13) zum Extrudieren des nicht granulierten Einfüllmaterials (5) von der zweiten Seite (12) der Trägerschicht (1) umfasst, und wobei die verstärkten Teile (7) der Basisfasern (3) und Grasfasern (2) eine widerstandsfähige und wasserdurchlässige Schicht (8) bilden, die mit der Trägerschicht verbunden ist und auf der sich die Grasfasern nach oben erstrecken.

2. Kunstrasen nach Anspruch 1, wobei die Basisfasern (3) und Grasfasern (2) wechselseitige Kontaktstellen (9) aufweisen, und wobei die Beschichtung (6) die verstärkten Teile (7) der Basisfasern (3) und Grasfasern an den Kontaktstellen (9) miteinander verbindet.

3. Kunstrasen nach Anspruch 1 oder 2, wobei das Elastomer Silikon, Styrol-Butadien-Kautschuk, Polyacrylkautschuk oder Polyurethan ist.

4. Kunstrasen nach Anspruch 1 bis 3, wobei die Höhe (10) der widerstandsfähigen und wasserdurchlässigen Schicht (8) im Bereich von 2 bis 50 Millimetern, vorzugsweise im Bereich von 5 bis 30 Millimetern, und besonders bevorzugt im Bereich von 10 bis 30 Millimetern liegt.

5. Kunstrasen nach Anspruch 1 bis 4, wobei sich die Grasfasern (2) zwischen 5 und 25 Millimeter auf der widerstandsfähigen und wasserdurchlässigen Schicht (8) nach oben erstrecken.

6. Kunstrasen nach Anspruch 1 bis 5, wobei die Fasern aus Filamenten gebildet sind und die Anzahl der Filamente pro Quadratmeter zwischen 90000 bis 350000 liegt.

7. Verfahren zur Herstellung eines Kunstrasens, umfassend die Schritte:
- Bereitstellen einer Trägerschicht (1) mit einer offenen Netzstruktur, umfassend eine erste Seite (11), eine zweite Seite (12) gegenüberliegend zur ersten Seite (11) und eine Vielzahl von Löchern,
- Anheften von Polgarn (14) in Abständen (15) an der ersten Seite (11) der Trägerschicht (1), um Kunstgrasfasern (2) bereitzustellen, die sich im Gebrauch von der Trägerschicht (1) nach oben erstrecken,
- Anheften von Polgarn (14) mit Abständen (15) an der ersten Seite (11) der Trägerschicht (1), um Kunstbasisfasern (3) bereitzustellen, die sich im Gebrauch von der Trägerschicht (1) nach oben erstrecken, **dadurch gekennzeichnet, dass** das nicht granulierte Einfüllmaterial (5), umfassend Elastomer, von der zweiten Seite (12) des Trägermaterials durch die Löcher (13) hindurch in der Trägerschicht (1) in die Räume (16) zwischen den Grasfasern (2) und Basisfasern (3) hinein extrudiert wird, so dass das nicht granulierte Einfüllmaterial (5) als eine Beschichtung (6) derart auf jede Faser (2, 3) aufgetragen wird, dass ein Teil der Länge der Grasfasern (2) und zumindest einen Teil der Länge der Basisfasern (3) bedeckt und dadurch die Fasern (2, 3) verstärkt werden, wobei die verstärkten Teile (7) der Basisfasern (3) und Grasfasern (2) eine widerstandsfähige und wasserdurchlässige Schicht (8) bilden, die an der Trägerschicht (1) befestigt ist und auf der sich die Grasfasern (2) nach oben erstrecken.

8. Verfahren zur Herstellung eines Kunstrasens nach Anspruch 7, wobei die Basisfasern (3) und Grasfasern (2) wechselseitige Kontaktstellen (3) aufweisen, und wobei die Beschichtung (6) die verstärkten Teile (7) der Basisfasern (3) und Grasfasern (2) an den Kontaktstellen miteinander verbindet.

9. Verfahren nach Anspruch 7 oder 8, wobei flüssiges Elastomer von der zweiten Seite (12) der Trägerschicht (1) durch die Löcher (13) hindurch in der Trägerschicht (1) in die Räume (16) zwischen den Grasfasern (2) und Basisfasern (3) hinein extrudiert wird, und das Elastomer ausgehärtet oder vulkanisiert wird, um die widerstandsfähige und wasserdurchlässige Schicht (8) aus verstärkten Fasern (2, 3) zu bilden.

10. Verfahren nach Anspruch 9, wobei das Elastomer Silikon, StyrolButadien-Kautschuk, Polyacrylkautschuk oder Polyurethan ist.

11. Verfahren nach Anspruch 7 bis 10, wobei die Höhe (10) der widerstandsfähigen und wasserdurchlässigen Schicht (8) in einem Bereich von 2 bis 50 Millimetern, vorzugsweise in einem Beriech von 5 bis 30 Millimetern, und besonders bevorzugt in einem Bereich von 10 bis 30 Millimetern liegt.

12. Verfahren nach Anspruch 7 bis 11, wobei sich die Grasfasern (2) zwischen 5 bis 25 Millimetern auf der widerstandsfähigen und wasserdurchlässigen Schicht (8) nach oben erstrecken.

13. Verfahren nach Anspruch 7 bis 12, wobei die Fasern aus Filamenten gebildet sind und die Anzahl der Filamente pro Quadratmeter zwischen 90000 bis 350000 liegt.

## Revendications

1. Gazon artificiel comprenant un support (1) de structure de réseau ouverte, une pluralité de fibres d'herbe artificielle (2) et une pluralité de fibres de base artificielle (3), dans lequel lesdites fibres d'herbe (2) et de base (3) sont attachées au support (1) et s'étendent vers le haut depuis le support (1) lors de l'utilisation, et dans lequel le support (1) comprend un premier côté (11) et un second côté (12) opposé au premier côté (11) et opposé aux fibres d'herbe (2) et de base (3) **caractérisé en ce que** les fibres d'herbe (2) et de base (3) sont renforcées par un matériau de remplissage non granulaire (5), qui comprend un élastomère, en tant que revêtement (6) sur chaque fibre (2, 3) et couvrant une partie de la longueur des fibres d'herbe (2) et au moins une partie de la longueur des fibres de base (3), et dans lequel le support (1) comprend des trous (13) pour extruder le matériau de remplissage non granulaire (5) depuis le second côté (12) du support (1) et dans lequel les parties renforcées (7) des fibres de base (3) et d'herbe (2) forment une couche élastique et perméable à l'eau (8) qui est attachée au support (1) et par-dessus laquelle s'étendent les fibres d'herbe (2).

2. Gazon artificiel selon la revendication 1, dans lequel les fibres de base (3) et d'herbe (2) ont des points de contact mutuels (9) et dans lequel le revêtement (6) lie les parties renforcées (7) des fibres de base (3) et d'herbe (2) ensemble au niveau des points de contact (9).

3. Gazon artificiel selon la revendication 1 ou 2, dans lequel l'élastomère est de la silicone, du caoutchouc de butadiène-styrène, du caoutchouc polyacrylique ou du polyuréthane.

4. Gazon artificiel selon les revendications 1 à 3, dans lequel la hauteur (10) de la couche élastique et perméable à l'eau (8) fait de 2 à 50 millimètres, préférentiellement de 5 à 30 millimètres et le plus préférentiellement de 10 à 30 millimètres.

5. Gazon artificiel selon les revendications 1 à 4, dans lequel les fibres d'herbe (2) s'étendent de 5 à 25 millimètres au-dessus de la couche élastique et perméable à l'eau (8).

6. Gazon artificiel selon les revendications 1 à 5, dans lequel les fibres sont constituées de filaments et le nombre de filaments par mètre carré est de 90000 à 350000.

7. Procédé de fabrication d'un gazon artificiel, comprenant les étapes de :
- fourniture d'un support (1) de structure de réseau ouverte comprenant un premier côté (11), un second côté (12) opposé au premier côté (11), et une pluralité de trous (13),
- fixation de fils de velours (14) à intervalles espacés (15) sur le premier côté (11) du support (1) pour fournir des fibres d'herbe artificielle (2) s'étendant vers le haut depuis le support (1) lors de l'utilisation,
- fixation de fils de velours (14) à intervalles espacés (15) sur le premier côté (11) du support (1) pour fournir des fibres de base artificielle (3) s'étendant vers le haut depuis le support (1) lors de l'utilisation, **caractérisé en ce qu'**un matériau de remplissage non granulaire (5) comprenant un élastomère est extrudé à partir du second côté (12) du support (1) à travers les trous (13) dans le support (1) dans les espaces (16) entre les fibres d'herbe (2) et fibres de base (3) de telle sorte que le matériau de remplissage non granulaire (5) est appliqué en tant que revêtement (6) sur chaque fibre (2, 3) d'une manière telle qu'il couvre une partie de la longueur des fibres d'herbe (2) et au moins une partie de la longueur des fibres de base (3) et renforce ainsi lesdites fibres (2, 3), dans lequel les parties renforcées (7) des fibres de base (3) et d'herbe (2) forment une couche élastique et perméable à l'eau (8) qui est fixée au support (1) et par-dessus laquelle s'étendent les fibres d'herbe (2).

8. Procédé de fabrication d'un gazon artificiel selon la revendication 7, dans lequel les fibres de base (3) et d'herbe (2) ont des points de contact mutuels (9) et dans lequel le revêtement (6) lie les parties renforcées (7) des fibres de base (3) et d'herbe (2) ensemble au niveau des points de contact (9).

9. Procédé selon la revendication 7 ou 8, dans lequel un élastomère fluide est extrudé à partir du second côté (12) du support (1) à travers les trous (13) dans le support (1) dans les espaces (16) entre les fibres d'herbe (2) et de base (3), et l'élastomère est durci ou vulcanisé pour former la couche élastique et perméable à l'eau (8) de fibres renforcées (2, 3).

10. Procédé selon la revendication 9, dans lequel l'élastomère est de la silicone, du caoutchouc de butadiène-styrène, du caoutchouc polyacrylique ou du polyuréthane.

11. Procédé selon les revendications 7 à 10, dans lequel la hauteur (10) de la couche élastique et perméable à l'eau (8) fait de 2 à 50 millimètres, préférentiellement de 5 à 30 millimètres et le plus préférentiellement de 10 à 30 millimètres.

12. Procédé selon les revendications 7 à 11, dans lequel les fibres d'herbe (2) s'étendent de 5 à 25 millimètres au-dessus de la couche élastique et perméable à l'eau (8).

13. Procédé selon les revendications 7 à 12, dans lequel les fibres sont constituées de filaments et le nombre de filaments par mètre carré est de 90000 à 350000.
